

# United States Patent Office

3,314,837

Patented Apr. 18, 1967

1

3,314,837

HYDRAZINE BASED SOLID PROPELLANTS  
Henry Philip Heubusch, Buffalo, N.Y., assignor to  
Bell Aerospace Corporation  
No Drawing. Filed Mar. 20, 1964, Ser. No. 353,601  
3 Claims. (Cl. 149—36)

This invention relates to new and useful energy generators and more particularly to that class of energy generators generally known as solid monopropellants of the single compound type, this application being a continuation-in-part of my copending application Ser. No. 835,387 filed Aug. 24, 1959, now abandoned.

There is today a great need for more powerful, stable and generally more easily handled gas generators, particularly for use as propellants in the rocketry field, and also for use in improved pyrotechnics and explosives.

At the present stage of development the propellants being used fall broadly into two categories, liquids and solids. The liquids have the advantage of inherent high energy but the disadvantage of being difficult to handle due to high corrosiveness, toxicity, and extremely high chemical activity. The solid propellants, or gas generators, have for some time been recognized as being more desirable from the standpoint of handling characteristics, being inherently more stable but up to now no solid fuel has been found which approximates the energy levels obtainable by the use of liquid fuels.

Of the solid fuel developments, the most success has been obtained with composite types, which generally comprise a physical mixture of an oxidizing salt and a fuel-binder. However, this method is limited by the fact that the ingredients which lend themselves to this type of formulation are of relatively low energy level and that the optimum energy level of the more powerful of the available ingredients cannot be obtained because the ingredients cannot be satisfactorily combined in the exact proportion which would give maximum energy output. It will be apparent that there is still a great need for more controllable, safer, and otherwise improved high energy gas generators which combine the respective advantages of the known liquid and solid generators. The advantages gained therefrom will be equally as useful in the explosive and pyrotechnic fields as for propellants.

It is therefore an object of this invention to provide methods for the production of new and useful gas generators.

It is another object of this invention to provide new and useful propellant compositions for use in reaction motors and the like.

Still another object of this invention is to provide new and useful polymeric materials which give outstanding thrust energy levels when used as fuels.

According to the present invention, polymers are formed which contain an amino group having an inorganic oxidizing acid attached thereto with such amino group being pendant from a nitrogen atom contained within the polymeric chain. Basically, there are three systems according to the present invention; one in which a polymer having the above characteristic is first formed by heating a strained ring hydrazine derivative, whereafter an inorganic oxidizing acid is added to the polymer to attach to the pendant amino groups; one in which a polymeric salt having the above characteristics is formed in situ from a starting mixture of an unsaturated hydrazine derivative and an inorganic oxidizing acid; and one in which the polymeric salt having the above characteristics is formed in situ from a starting mixture of a hydroxy alkyl hydrazine compound, a polyfunctional compound, and an inorganic oxidizing acid.

The oxidizing acid may be perchloric acid, nitric acid, sulfuric acid, phosphoric acid and mixtures thereof; al-

2

though it is preferred to use perchloric acid due to its richness in oxygen.

In addition, the first system mentioned above, polymeric salts obtained from strained ring (3-5 members) hydrazine derivatives, is preferred since the process, in general, is the simplest and most economical of the three. To illustrate this system, such derivatives as N-amino-ethyleneimine (three membered ring), 3-amino-2-oxazolidinone (five membered ring), and the like may be used as the starting compound. For example, the polymer polyethylene hydrazine may be formed by decarboxylation of 3-amino-2-oxazolidinone, the basic recurring unit of such polymer having the following structural formula:



Although the method of making polyethylene hydrazine forms, per se, no part of the present invention, a preferred method for obtaining this polymer is by the decarboxylation of 3-amino-2-oxazolidinone. Specifically, 3-amino-2-oxazolidinone is decarboxylated by continued heating at 210° C. until the evolution of carbon dioxide has diminished as is indicated by repeated collapsing of the foaming product. At this point, the product is cooled quickly to room temperature and, thereafter, the product is maintained at a temperature of 105° C. for twenty-four hours and under a vacuum of 0.1 mm. of mercury. The resultant polymer, polyethylene hydrazine, has a molecular weight of about 700, a density of 1.3 grams per cc. and a softening point of about 90° C.

### Example I

Polyethylene hydrazine, which may be prepared as specified above, is formed into a slurry with a suitable solvent such as methanol, ethanol, or the like, it being preferred that the amount of solvent be minimized and that the same be present only in such amount as to provide a vehicle for polyethylene hydrazine. While maintaining the temperature of the products below 25° C., perchloric acid is added to the above slurry, with stirring. The perchloric acid is added in the ratio of 2.0 moles of perchloric acid per 1.0 mole polyethylene hydrazine, the time required for the addition of the perchloric acid being determined by the temperature of the mixture, the same being maintained below 25° C. as specified above. The temperature may be maintained by any suitable external cooling arrangement sufficient to remove the heat of the reaction rapidly enough as to control the temperature as aforesaid.

After all of the perchloric acid has been added, the reaction product is brought to room temperature and agitated to produce a pale yellow solid. This product may be isolated by filtration followed by washing with methanol and ether and drying in vacuo. The product has a density of about 1.70 grams per cc. and exhibits a burning rate of about 4 inches per second at 1000 p.s.i.g. and its combustion efficiency exceeds 90%. The product reaches an auto-ignition point at about 120° C. and reaches an average molecular weight of 520. Investigation shows that the resultant polymer is characterized, within the basic recurring unit of the polymer, by a pendant amino group having the perchloric acid attached thereto and that the polymer contains approximately 20% chloride and has the following general structural formula:



in which  $x$  is approximately 0.8 and  $n$  is 4.

Although the monopropellant possesses a high burning rate as described above, its sensitivity to impact is com-

## 3

parable to conventional operational propellants. Specifically, the present monopropellant exhibits reaction to the impact of an 80 oz. weight dropped from a height of about 6 inches not more than one out of ten times. In the preparation of the monopropellant as specified hereinabove, the amount of agitation at room temperature subsequent to the initial reaction between the perchloric acid and polyethylene hydrazine may be as little as 0.2 hour. Tests indicate no difference in the monopropellant obtained after 0.2 hour of agitation and that obtained after 20 hours of agitation, indicating that the monopropellant according to the present invention may be commercially prepared in continuous fashion.

## Example II

Example I is repeated except that nitric acid is substituted for perchloric acid.

## Example III

Example I is repeated except that sulfuric acid is substituted for perchloric acid.

The polymeric salts of Examples II and III yield results similar to those obtained in Example I, demonstrating the practicality of using different inorganic oxidizing acids. As stated hereinbefore, the use of perchloric acid is preferred due to the high oxygen content of this particular acid.

In the second system mentioned above (polyenes), the unsaturated hydrazine derivative must contain at least one double bond between carbon atoms, necessitating that the unsaturated compound contain at least two carbon atoms while practical considerations involving availability of starting compounds dictates that the unsaturated derivative may contain up to eight carbon atoms.

## Example IV

To one mole of an aqueous solution of monomethylallyl hydrazine  $\text{CH}_2=\text{C}(\text{CH}_3)\text{CH}_2\text{NHNH}_2$  is added one mole of sulfuric acid. The resulting solution is vacuum distilled at 70° C. and 0.3 p.s.i.a. for 2 hours to remove water; the temperature is then increased to about 125° C. at a pressure of 3 p.s.i.a. for several hours until a brown, thermoplastic polymer results.

## Example V

To one mole of an aqueous solution of unsymmetrical diallyl hydrazine is added one mole of sulfuric acid. The resulting solution is refluxed at atmospheric pressure for 8 hours and the product is isolated by vacuum distillation at elevated temperature. Specifically, starting from 100° C. and 0.2 p.s.i.a., the temperature is gradually increased to 190° C. until a red-brown thermoplastic polymer is formed.

## Example VI

Example V is repeated except that nitric acid is substituted for the sulfuric acid, yielding similar results.

It is interesting to note that in Examples IV, V and VI, the inorganic oxidizing acid acted as a catalyst as well as providing the oxidizer function in the monopropellant combination. Moreover, attempts to effect polymerization of the unsaturated hydrazine compound were unsuccessful when conventional catalysts such as benzoyl peroxide, tertiary butyl hydrogen peroxide, ferric chloride and the like were used.

The third class mentioned above (polyesters) involves the condensation of a hydroxy alkyl hydrazine with a polyfunctional compound selected from the group consisting of  $(\text{CH}_2)_x(\text{COOH})_2$ ;  $(\text{CH}_2)_x(\text{COY})_2$ ;  $(\text{CH}_2)_x(\text{COOR})_2$  and  $(\text{CH}_2)_x(\text{CO})_2\text{O}$ , where  $x$  is 0 to

8, Y is a halogen and R is an alkyl group, in the presence of an inorganic oxidizing acid. That is to say, the polyfunctional compounds may be dibasic acids  $[(\text{CH}_2)_x(\text{COOH})_2]$ ; the corresponding acid halides of these dibasic acids; esters of these dibasic acids and alkyl alcohols; and corresponding anhydrides of these dibasic acids, where  $x$  is 0 to 8.

## Example VII

To one mole of an aqueous solution of unsymmetrical diethanol hydrazine  $(\text{HOCH}_2\text{CH}_2)_2\text{NNH}_2$  is added one mole of oxalic acid and one mole of sulfuric acid. The resulting solution is refluxed at atmospheric pressure for 8 hours, yielding a red liquid. Water is then removed by vacuum distillation at 100° C. and 0.2 p.s.i.a. until a dark red thermoplastic polymer forms.

## Example VIII

Example VII is repeated except that unsymmetrical diisopropanol hydrazine  $(\text{H}_3\text{CCH}(\text{OH})\text{CH}_2)_2\text{NNH}_2$  is substituted for the unsymmetrical diethanol hydrazine. A brown thermoplastic polymer results.

It is to be understood that certain changes and modifications may be made without departing from the spirit of the invention or the scope of the following claims.

I claim:

1. A method of making a polymer characterized by its ability to evolve sufficient quantity of gaseous products as to render the polymer useful as a rocket propellant and the like, which comprises forming a slurry of polyethylene hydrazine and a solvent therefor, adding perchloric acid to said slurry in about the ratio of 2 moles perchloric acid to 1 mole of polyethylene hydrazine, while maintaining the temperature of the mixture below about 25° C., agitating the mixture at room temperature and recovering the solid formed.

2. Polyethylene hydrazine perchlorate useful as a solid propellant characterized by its high burning rate combined with high stability and relative insensitivity to impact, having the general structure:



where  $x$  is about 0.8 and  $n$  is an integer.

3. A method of making a polymer characterized by its ability to evolve sufficient quantity of gaseous products as to render the polymer useful as a rocket propellant and the like, which comprises forming a slurry of polyethylene hydrazine and a solvent therefor, adding an inorganic oxidizing acid to said slurry in about the ratio of 2 moles of acid to 1 mole of polyethylene hydrazine, while maintaining the temperature of the mixture below about 25° C., agitating the mixture at room temperature and recovering the solid formed.

## References Cited by the Examiner

## UNITED STATES PATENTS

3,211,720 10/1965 Heubusch ----- 149-36 X

CARL D. QUARFORTH, Primary Examiner.

REUBEN EPSTEIN, LEON D. ROSDOL, Examiners.

L. A. SEBASTIAN, Assistant Examiner.